

## 1 BEST AVAILABLE COPY

## 2

3,298,774

## DYEING POLYAMIDE FIBERS

Charles Soiron, Riehen, Switzerland, Hans Rafael, Weil am Rhine, Germany, and Walter Stockar, Munchenstein, Switzerland, assignors to J. R. Geigy A.-G., Basel, Switzerland

No Drawing. Filed July 19, 1963, Ser. No. 296,390  
Claims priority, application Switzerland, July 31, 1962,

9,157/62

18 Claims. (Cl. 8—74)

This invention relates to improvements in dyeing polyamide fibers as well as, as industrial product, the dyed polyamide fibers treated according to the invention.

Hitherto, wool and other polyamide fibers including nylon and the like synthetic polyamide fibers which had been dyed with reactive dyestuffs containing per molecule at least one substituent which can be split off as an anion during the dyeing and/or after-treatment of the dyed fibers, had to be subjected to an after-treatment in an aqueous basic medium of a pH of preferably about 7.5 or higher which contains, for example, sodium hydroxide, sodium carbonate, or preferably ammonia or hexamethylenetetramine as the basic agent.

This known alkaline after-treatment, which serves to fix on the fibers still unreacted reactive dyestuff present in the dyed goods, suffers from the drawback that the polyamide fibers can be injured by the alkaline medium and particularly by a subsequent drying step if the same is carried out directly on the after-treated fibers.

Therefore, in the known dyeing methods the after-treatment with an alkaline medium is followed usually by a further treatment in an acid medium prior to final drying of the dyed fibers.

Another drawback of the after-treatment with alkaline agents such as ammonia or hexamethylenetetramine resides in the tendency of the alkaline bath to remove at least part of the still unreacted dyestuff from the fibers, whereby an exact control of the shade of the fixed dyeings is made very difficult.

It is, therefore, an object of the present invention to provide in a process of dyeing polyamide fibers with reactive dyestuffs of the type described, an after-treatment of the dyed fibers for the purpose of fixing still unreacted residual dyestuff or the fibers, which after treatment does not injure the fibers, permits of dyeing the after-treatment fibers directly without further intermediate treatments, and allows for a more exact control in producing a desired shade.

These objects are attained by the treatment according to the invention, which comprises; as an after-treatment in a process for dyeing polyamide fibers, after heating and thereby reacting these fibers in an acid dye-bath with a reactive dyestuff which contains at least one mobile substituent capable of being split off as anion, and after substantial exhaustion of the dye-bath,

(I) Adding to the dye-bath still containing the fibers a condensation product of

(a) A naphthalene sulfonic acid, in particular a mono- to trisulfonic acid, and preferably naphthalene-2-monosulfonic acid, or a 1,2,3,4-tetrahydronaphthalene sulfonic acid,

(b) From about 0.5 to 1.5, and preferably from 0.8 to 1.2 part by weight, per part by weight of (a), of a compound of the formula

$\text{HO-phenylene-SO}_2\text{-phenylene-OH}$ , preferably 4,4'-dihydroxydiphenylsulfone, and

(c) From about 0.1 to 0.2, and preferably 0.1 part by weight, per part by weight of (a), of formaldehyde, in aqueous, preferably about 30%-solution, and

(II) Heating the dye-bath and the fibers therein for a short time, about 10 to 60, and preferably 15 to 30

minutes at a temperature of about 50° to 100°, and preferably 60° to 85° C.

As polyamide fiber these of natural origin above all wool and silk, as well as synthetic polyamide fibers such as the various kinds of nylon, e.g. nylon 6, nylon 66 and nylon 11 (Rilsan), are suitable for the after-treatment according to the invention.

The polyamide fibers are dyed by known methods in a dyestuff solution which, in addition to the known dyestuffs, can also contain the auxiliaries usual in wool dyeing, for example, salts such as sodium sulphate or ammonium sulphate and/or dilute acids, e.g. acetic or formic acid and/or wetting agents, e.g. condensation products of fatty acids having at least 8 carbon atoms with lower alkanolamines such as are described in U.S. Patent 2,089,212.

After the dyestuff has been drawn onto the fibers and the dyebath is satisfactorily exhausted, the dyed goods are after-treated according to the invention in the same bath as that in which they were dyed, by adding the condensation product, preferably in dissolved form, alone or together with other additives usual in textile dyeing, and moreover, preferably in condition with an acid, especially acetic or formic acid or their water soluble salts, to the at least slightly cooled dyebath which has a pH of about 4 to 5.5, and preferably 4.5 to 5. Acetic acid is preferred.

The aforesaid condensation products which are suitable for use in the treatment according to the invention are produced as described in German Patent 611,671, issued April 5, 1935.

The content of these condensation products in the treatment liquor should be about 0.5 to 3 grams per liter.

The reactive dyestuffs which can be used according to the invention can be of the most various classes of dyestuffs. Advantageously they are the nitro, azo, anthraquinone and phthalocyanine dyestuff classes which are distinguished by their stability. They contain water solubilizing, acid salt-forming groups, mainly sulphonate acid groups, also they may contain carboxyl groups or sulphamyl groups, in the latter case, also acylated sulphamyl groups among others, e.g. disulphimide and carbonyl sulphimide groups. The advantages attainable according to the invention are particularly impressive if reactive dyestuffs usual for the fast dyeing of cellulose are used, which dyestuffs contain several sulfonic acid groups, for example, 2 to 4 per dyestuff molecule. Thus, the dyestuffs used according to the invention are, for example, nitro diaryl amino sulphonate acids, metal-free mono- and poly-azo dyestuffs, heavy metal-containing, for example, chromium or cobalt containing, o,o'-dihydroxy, o-hydroxy-o'-carboxy, and o-hydroxy-o'-amino monoazo and disazo dyestuffs, copper containing formazane dyestuffs, 1-amino-4-phenylamino-anthraquinone dyestuffs, copper phthalocyanines having substituted sulphamyl groups, all of which preferably contain at least two sulphonate acid groups. Radicals of strong acids are chiefly used as mobile substituents which can be split off as anion, in particular halogen atoms, of these preferably chlorine, or also bromine or fluorine, the mobility of which is due, for example, to the bond to  $\beta$ -carbon atoms in negatively substituted organic radicals, to carbon atoms of nitrogen heterocycles of aromatic character which are adjacent to a tertiary ring nitrogen atom, in this case, preferably 6-membered heterocycles having at least two tertiary ring nitrogen atoms; or aromatically bound halogen atoms in o- or p-position to one (or more) electrophilic group(s) e.g. the  $\text{NO}_2$  or  $\text{SO}_2$  group, in particular, mainly fluorine or chlorine atoms. Additional examples of mobile substituents which can be split off as anion are: the radical of sulphuric acid in sulphated  $\beta$ -hydroxyalkyl compounds, e.g. in sulphated  $\beta$ -hydroxyalkyl

sulphonyl and sulphamyl groups, or the radical of hydroxyaryl compounds in O-aryl urethane groups.

Dyestuffs usable according to the invention contain the substituent which can be split off as anion, for example, in the form of  $\beta$ -chloro- or  $\beta$ -bromo-fatty acid amide groups, in this case particularly  $\beta$ -chlorocrotonic acid amide or  $\beta$ -bromopropionic acid amide groups, in the form of fluoro- or chloro-nitrobenzoyl-amino groups or fluoro or chloro-nitrobenzene sulphonylamino groups in which the fluorine or chlorine atoms are in the o- or/and p-position to the nitro group(s), and preferably in the form of chloro- or bromo-diazinylamino groups or chloro- or bromo-triazinylamino groups, in which case particularly monochloro- or dichloro-s-triazinylamino groups and, preferably, di- or trichloropyrimidylamino groups. Dyestuffs having at least one and not more than two di- or tri-halogen pyrimidylamino groups and at least two and maximally five sulphonic acid groups are preferred in the dyeing processes according to the invention.

An advantage of the treatment according to the invention over the known processes is the elimination of an alkaline after-treatment with, for example ammonia or hexamethylenetetramine. This advantage becomes most apparent in the dyeing of wool which is sensitive to alkali, as the danger of injury to the fibers inherent in the alkaline after-treatment is avoided.

Moreover, the control of producing the desired shade more exactly is facilitated since changes in shade due to shifting of the pH of the dyeing medium from acid to alkaline and possibly back to acid are avoided.

Dyeings or prints on polyamide fibers attained according to the invention are distinguished by pure, strong and even shades and good fastness properties. In particular, they have remarkable wet fastness properties, for example fastness to water, washing, milling and perspiration, and particularly to sea water.

The following non-limitative examples illustrate the invention. Where not otherwise stated, parts and percentages are given by weight unless stated otherwise. The relationship of parts by weight to parts by volume is as that of grams to cubic centimeters. The temperatures are given in degrees centigrade.

#### Example 1

100 parts of wool are dyed in 4000 parts of a dye liquor

45 which contains the following agents: 4 parts of a dyestuff of the formula

5

10

20

25

30

35

40

45



0.5 part of a condensation product of 1 mol of oleic acid and 2 mols of diethanolamine produced as described in U.S. Patent No. 2,089,212 and 4 parts of 80% acetic acid.

The goods are introduced into the liquor at 50°, dyeing is performed for 10 minutes at this temperature, the bath is brought to the boil within 30 minutes and dyeing is continued at the boil for 45 minutes.

The dyebath is then allowed to cool to about 60–80° whereupon 100 parts of a solution of 30 g. per liter of a condensation product of formaldehyde with dihydroxydiphenyl sulphone and naphthalene sulphonic acids are added thereto. The production of the condensation product is described below.

This mixture is left for 15–20 minutes at about 60–80°. The liquor is then cooled, the wool is well rinsed with water, squeezed out and dried.

Valuable vivid blueish red dyeings are obtained in this manner. The dyeings are very wet fast.

The condensation product mentioned is obtained as follows:

100 parts of the sulfonating mixture, obtained by heating for several hours at 140–160°, 520 parts of naphthalene and 560 parts of concentrated sulphuric acid until water solubility is attained, are heated for about 1 hour at 105–110° with 100 parts of a dihydroxydiphenyl sulphone, 50 parts of water and 45 parts of formaldehyde (30%). The dihydroxydiphenyl sulphone is obtained by heating 540 parts of phenol and 180 parts of 60% oleum for 3 hours at 170–180° and distilling off excess phenol. If, instead of the dyestuff given in the example, the dyestuffs mentioned in column 2 of the following table are used and otherwise the procedure described is followed, then wool dyeings as given in column 3 are obtained.

TABLE

| No. | Dyestuff | Shade on wool    |
|-----|----------|------------------|
| 1   |          | Greenish yellow. |
| 2   |          | Reddish yellow.  |
| 3   |          | Red.             |

TABLE—Continued.

| No. | Dyestuff                                                                                                                                       | Shade on wool   |
|-----|------------------------------------------------------------------------------------------------------------------------------------------------|-----------------|
| 4   |                                                               | Blue.           |
| 5   |                                                               | Scarlet.        |
| 6   |                                                               | Orange.         |
| 7   | <br>(wherein Cu-Phtc. is the copper phthalocyanine radical) | Turquoise blue. |
| 8   |                                                             | Bordeaux.       |
| 9   |                                                             | Blue.           |
| 10  |                                                             | Black.          |

TABLE—Continued.

| No.     | Dyestuff | Shade on wool    |
|---------|----------|------------------|
| 11----- |          | Orange.          |
| 12----- |          | Greenish yellow. |

*Example 2*

100 parts of nylon 6 are dyed in 4000 parts of a dye liquor which contains 1.5 parts of a dyestuff of the formula



and 1 part of 80% acetic acid.

The goods are introduced at 40°, dyeing is performed for 10 minutes at this temperature, the bath is brought to the boil within 30 minutes and dyeing is continued for 45 minutes at the boil.

The dyebath is then allowed to cool to about 60-80° and then 100 parts of a solution of 30 g. per liter of the formaldehyde/dihydroxydiphenylsulphone/naphthalene sulfonic acids condensation product mentioned in paragraph 3 of Example 1 is added.

This mixture is left for 15-20 minutes at about 60-80°. The bath is then cooled, the nylon is well rinsed with water, squeezed out and dried.

In this way valuable greenish yellow, very wet fast dyeings are obtained.

We claim:

1. In a process for dyeing polyamide fibers which process comprises heating and thereby reacting, in an acid dyebath, said fibers with a reactive dyestuff which contains at least one mobile substituent which is split off as anion, the improvement comprising  
 60 (I) adding to the dyebath which still contains the fibers, after the dye has drawn onto the latter, a condensation product of  
 (a) a member selected from the group consisting of a naphthalene sulfonic acid and a 1,2,3,4-tetrahydronaphthalene sulfonic acid,  
 (b) from about 0.5 to 1.5 parts by weight of a compound of the formula  

$$\text{HO—phenylene—SO}_2\text{—phenylene—OH}$$
 65 per part by weight of (a), and  
 (c) from about 0.1 to 0.2 part by weight of formaldehyde per part by weight of (a), in aqueous solution, and  
 70  
 75  
 80  
 85  
 90  
 95  
 100  
 105  
 110  
 115  
 120  
 125  
 130  
 135  
 140  
 145  
 150  
 155  
 160  
 165  
 170  
 175  
 180  
 185  
 190  
 195  
 200  
 205  
 210  
 215  
 220  
 225  
 230  
 235  
 240  
 245  
 250  
 255  
 260  
 265  
 270  
 275  
 280  
 285  
 290  
 295  
 300  
 305  
 310  
 315  
 320  
 325  
 330  
 335  
 340  
 345  
 350

product of fatty acid of at least 8 carbon atoms and lower alkanolamine is added to the dyebath as the dyeing auxiliary.

17. The improvement described in claim 16 wherein the condensation product of oleic acid and diethanolamine in a molar ratio of 1:2 is used as the dyeing auxiliary.

18. The improvement described in claim 16 wherein said dyeing auxiliary is added in an amount of about 0.5% calculated on the weight of the fibers being dyed.

## References Cited by the Examiner

## UNITED STATES PATENTS

- 2,623,806 12/1952 Fuchs ----- 8-21  
5 3,118,723 1/1964 Harding ----- 8-54 X

NORMAN G. TORCHIN, Primary Examiner.

T. J. HERBERT, Assistant Examiner.